

## UNITED STATES PATENT OFFICE

2,010,822

## MANUFACTURE OF CELLULOSE ACETATE

Carl J. Malm, Rochester, N. Y., assignor to Eastman Kodak Company, Rochester, N. Y., a corporation of New York

No Drawing. Application September 16, 1931,  
Serial No. 563,230

3 Claims. (Cl. 260—101)

This application is a continuation-in-part of my co-pending application Serial No. 336,922, filed February 1, 1929, now U. S. Patent No. 1,908,525.

5 The present invention relates to the pretreatment of cellulose with acetic acid and a chlorinated aliphatic hydrocarbon and then esterifying the pretreated cellulose.

One object of my invention is to utilize the 10 bath in which cellulose has been pretreated, to form the subsequent esterification bath by merely adding esterifying ingredients to it after the pretreatment of the cellulose has been completed. The amount of chlorinated aliphatic hydrocarbon 15 which is employed in the pretreatment bath together with the organic acid is preferably the amount of the chlorinated hydrocarbon which is desired in the esterification bath so that there will be no waste of this ingredient by using an excess in the pretreatment and so that it will be 20 unnecessary to add more of this chlorinated hydrocarbon at any time after the pretreatment. Of course, if additional chlorinated hydrocarbon is preferred in certain cases, it may be added in 25 compatible amounts providing it does not interfere with the esterification.

The present invention is an improvement of the process disclosed in U. S. Patent No. 1,823,359 of H. LeB. Gray, which discloses a process of 30 acetylating cellulose in which the cellulose is pretreated with acetic acid and an acid catalyst, at the end of which treatment the mass of material is pressed until the ratio of acid to cellulose is approximately two to one. The cellulose is 35 then acetylated with a mixture of acetic anhydride and ethylene chloride.

I have now found a process of acetylating cellulose wherein the intermediate step of pressing out the pretreatment liquid is unnecessary between 40 the pretreatment and the esterification of the cellulose. For example by my invention the pressing operation between the pretreatment and acetylation of the Gray application is unnecessary and can be eliminated so that a considerable saving 45 in acetic acid which is necessary in any one operation may be effected.

I have found that the process described in the 50 Gray application, referred to above, may be improved by pretreating the cellulose with a mixture of acetic acid and a chlorinated hydrocarbon, such as chloroform, ethylene dichloride, methylene chloride, dichlorethylene, trichlorethylene, or carbon tetrachloride and then without pressing out any of the liquid absorbed from the 55 pretreatment bath, acetylating the pretreated cel-

lulose by adding the acetylating materials to the pretreatment batch. I have found that if the cellulose is pretreated with acetic acid together with a chlorinated hydrocarbon the acetic acid is evenly distributed throughout the cotton and a uniform and efficient pretreatment obtained. An acetylation catalyst, such as sulfuric acid may be added to the pretreatment mixture or it may be added to the acetic anhydride in the esterification step as desired, or it may even be present 10 as an impurity in some of the reagents employed.

As pointed out above, intermediate steps between the pretreatment and the esterification, such as for the removal of acetic acid are unnecessary in the performance of my invention.

15 The following example is an illustration of one embodiment of my invention:

About 25 lbs. of cotton are treated with a mixture of about 25 lbs. of acetic acid and 175 lbs. of ethylene chloride for about 4 hours at about 20 100° F. The mixture is then cooled to approximately 60° F. and then about 75 lbs. of 85% acetic anhydride containing about 1/2 lb. of sulfuric acid is added thereto. The temperature is then allowed to rise slowly to a maximum of 25 about 100° F. when a viscous clear solution is obtained denoting completion of the acetylation.

The reaction mixture or "dope" produced, which comprises cellulose acetate dissolved in acetic acid and ethylene chloride, is preferably 30 treated in a precipitating bath at a temperature at or above the boiling point of ethylene chloride. For example, the mass may be poured into water close to 100° C. whereupon the ethylene chloride evaporates and may be withdrawn and 35 condensed. The acetic acid is dissolved in the water and the cellulose acetate is precipitated.

Obviously, in cases where a chlorinated hydrocarbon, such as carbon tetrachloride (which acts as a precipitant when present in acetic acid in 40 an appreciable amount) is employed, in the pretreatment bath with acetic acid, it must be employed in restricted amounts. However, if one desires a fibrous acetylation process the amount of carbon tetrachloride need not be limited to 45 non-precipitating proportions, but may be employed in substantial amounts; equal parts of carbon tetrachloride and glacial acetic acid in the pretreatment is preferred when using that particular chlorinated hydrocarbon.

50 Other modifications of my invention such as its use in the production of esters having higher acid radicals, such as cellulose propionate, cellulose acetate butyrate, etc., or the use of other known acetylation catalysts will be obvious to 55

those skilled in the art and come within the contemplation of my invention.

I claim as my invention:

1. A process of acylating cellulose which comprises pretreating the cellulose with a bath comprising a fatty acid and ethylene chloride and subsequently adding a fatty acid anhydrid thereto.

2. A process of acylating cellulose which com-

prises pretreating the cellulose with a bath comprising acetic acid and ethylene chloride and subsequently adding a fatty acid anhydrid thereto.

3. A process of acylating cellulose which comprises pretreating the cellulose with a bath comprising a fatty acid and ethylene chloride and subsequently adding a fatty acid anhydrid together with a catalyst thereto.

CARL J. MALM.